# EUROPEAN PATENT APPLICATION

(11) **EP 0 304 113 A1**
(43) Date of publication of application: **22.02.1989**
(21) Application number: 88201675.1
(22) Date of filing: 03.08.1988
(51) Int. Cl.: H01F 1/04

(54) **Starting material for permanent magnets**

(30) Priority: 21.08.1987 NL 8701970
(71) Applicant: Philips Electronics N.V., 5621 BA Eindhoven (NL)
(72) Inventor: De Mooij, Dirk Bastiaan, NL-5656 AA Eindhoven (NL); Van Mens, Reinoud, NL-5656 AA Eindhoven (NL); Buschow, Kurt Heinz Jürgen, NL-5656 AA Eindhoven (NL)
(74) Representative: Pennings, Johannes

(57) **Abstract**

Hard-magnetic materials having a high crystal anisotropy on a carbide basis of the general formula (RE₁₋ₓNdₓ) Fe₁₄C, wherein
RE is a rare earth metal having an atomic number exceeding 61 and 0.50 ≦ x ≦ 0.80 have a comparatively high Curie-temperature.

## Description

The invention relates to a hard-magnetic material which comprises neodymium and iron.

A known material of this type is the Nd₂ Fe₁₄ B having a tetragonal crystal structure. It is known that a substitution of B by C in this compound leads to a greater anisotropy (see, for example, Journal de Physique Colloque C6, supplément au no. 9, T. 46, September, 1985, pages C6-305/308: "Magnetic anisotropy of Carbon Doped Nd₂Fe₁₄B" by Bolzoni, Leccabue, Pareti and Sanchez). It is stated in this article on page 306 that it was not possible to obtain the tetragonal phase when borium was replaced entirely by carbon.

It is the object of the invention to provide a hard-magnetic material having a great crystal anisotropy which comprises only carbon instead of boron and also a comparatively high content of neodymium.

It has been found that this object can be achieved by means of a substance of the following composition:
(RE₁₋ₓNdₓ) Fe₁₄C,
wherein RE is one or more rare earth metals having an atomic number exceeding 61 (for example Sm, Eu, Gd, Tb, Dy, Ho, Er, Tm, Lu) and
0.5 ≦ x ≦ 0.80.

It has been found that the magnetic properties decrease substantially if x < 0.5 or if x > 0.8.

In all the combinations a carbide having a tetragonal crystal structure is found. The Curie-temperature is between 500 and 600 K. The hard-magnetic materials according to the invention can be obtained in the conventional manner by fusing starting materials suitable for that purpose succeeded by an annealing treatment in a protective gas or another vacuum. A number of materials which were obtained in this manner are collected in the following table which also states the Curie-temperature and the annealing temperature.

**Table**

| Compound | Curie-temperature (K) | Annealing temperature (°C) |
|---|---|---|
| TbNdFe₁₄C | 560 | 850 |
| Tb_{0.5}Nd_{1.5}Fe₁₄C | 550 | 800 |
| Dy_{0.5}Nd_{1.5}Fe₁₄C | 545 | 850 |
| LuNdFe₁₄C | 530 | 850 |

The magnetic properties are comparable to those of materials on the basis of Nd₂Fe₁₄B or better. The absence of boron is an advantage since now poisonous volatile boron compounds cannot be formed in the preparation.

Magnets in the form of shaped bodies can be sintered from the resulting material after pulverisation in the manner conventional with Nd₂Fe₁₄B.

## Claims

1. A hard-magnetic material which comprises neodymium and iron, characterized in that the material has the composition (RE₁₋ₓNdₓ) Fe₁₄C, wherein RE is Sm, Eu, Gd, Tb, Dy, Ho, Er, Tm and/or Lu and
0.5 ≦ x ≦ 0.8.

2. A permanent magnet on the basis of a material as claimed in Claim 1.
